



US007527681B2

(12) **United States Patent**  
**Poole et al.**

(10) **Patent No.:** **US 7,527,681 B2**  
(b5) **Date of Patent:** **May 5, 2009**

(54) **ELECTROLESS COPPER AND REDOX COUPLES**

(75) Inventors: **Mark A. Poole**, Shrewsbury, MA (US); **Andrew J. Cobley**, West Midlands (GB); **Amrik Singh**, West Midlands (GB); **Deborah V. Hirst**, Nuneaton (GB)

(73) Assignee: **Rohm and Haas Electronic Materials LLP**, Marlborough, MA (US)

(\*) Notice: Subject to any disclaimer, the term of this patent is extended or adjusted under 35 U.S.C. 154(b) by 72 days.

(21) Appl. No.: **11/825,355**

(22) Filed: **Jul. 6, 2007**

(65) **Prior Publication Data**

US 2008/0038449 A1 Feb. 14, 2008

**Related U.S. Application Data**

(60) Provisional application No. 60/819,250, filed on Jul. 7, 2006.

(51) **Int. Cl.**

**C23C 18/38** (2006.01)  
**C23C 18/40** (2006.01)  
**B05D 5/12** (2006.01)  
**H05K 3/18** (2006.01)

(52) **U.S. Cl.** ..... **106/1.23**; 106/1.26; 427/97.9; 427/443.1

(58) **Field of Classification Search** ..... 106/1.23, 106/1.26; 427/97.9, 443.1

See application file for complete search history.

(56) **References Cited**

**U.S. PATENT DOCUMENTS**

4,002,786 A 1/1977 Hirohata et al.  
4,009,087 A 2/1977 Kardos et al.  
4,099,974 A 7/1978 Morishita et al.  
4,133,908 A 1/1979 Madsen  
4,192,764 A 3/1980 Madsen  
4,211,564 A 7/1980 Oka  
4,248,633 A 2/1981 Heijnen et al.  
4,303,443 A 12/1981 Miyazawa et al.  
4,371,397 A 2/1983 Honma et al.  
4,458,644 A 10/1985 Nakaso et al.  
4,557,762 A 12/1985 Nakaso et al.  
4,559,166 A 12/1985 Morinaga et al.  
4,563,217 A 1/1986 Kikuchi et al.  
4,695,505 A 9/1987 Dutkewych  
4,777,078 A 10/1988 Miyabayashi  
4,834,796 A 5/1989 Kondo et al.  
5,021,135 A 6/1991 Wilson et al.  
5,039,338 A 8/1991 Kondo et al.  
5,076,840 A 12/1991 Takita et al.  
5,358,992 A 10/1994 Dershem et al.

|                   |         |                             |
|-------------------|---------|-----------------------------|
| 5,419,926 A       | 5/1995  | Soltys                      |
| 5,425,873 A       | 6/1995  | Bladon et al.               |
| 5,620,961 A       | 4/1997  | Markovic et al.             |
| 5,789,507 A       | 8/1998  | Tanaka et al.               |
| 5,859,273 A *     | 1/1999  | Wilson et al. .... 556/148  |
| 5,897,692 A       | 4/1999  | Kotsuka et al.              |
| 5,965,211 A       | 10/1999 | Kondo et al.                |
| 6,107,426 A       | 8/2000  | Shibutani                   |
| 6,183,545 B1      | 2/2001  | Okuhama et al.              |
| 6,416,812 B1      | 7/2002  | Andricacos et al.           |
| 6,627,544 B2      | 9/2003  | Izumi et al.                |
| 6,660,071 B2      | 12/2003 | Yoshida et al.              |
| 6,664,122 B1      | 12/2003 | Andryuschenko et al.        |
| 6,805,915 B2      | 10/2004 | Itabashi et al.             |
| 6,855,378 B1      | 2/2005  | Narang                      |
| 7,291,217 B2 *    | 11/2007 | Phelps et al. .... 106/480  |
| 2002/0152955 A1   | 10/2002 | Dordi et al.                |
| 2003/0183120 A1   | 10/2003 | Itabashi et al.             |
| 2004/0104377 A1 * | 6/2004  | Phelps et al. .... 252/387  |
| 2004/0253450 A1   | 12/2004 | Seita et al. .... 428/411.1 |
| 2007/0071904 A1 * | 3/2007  | Yabe et al. .... 106/1.23   |
| 2008/0038450 A1 * | 2/2008  | Poole et al. .... 427/97.9  |
| 2008/0038451 A1 * | 2/2008  | Poole et al. .... 427/97.9  |
| 2008/0038452 A1 * | 2/2008  | Poole et al. .... 106/1.23  |

**FOREIGN PATENT DOCUMENTS**

|    |                   |        |
|----|-------------------|--------|
| EP | 1 411 147         | 4/2004 |
| GB | 1 397 091         | 7/1972 |
| JP | 1997316649 A      | 9/1997 |
| JP | 1998072677 A      | 3/1998 |
| JP | 2001148561 A      | 5/2001 |
| WO | WO 01/38604 A1    | 5/2001 |
| WO | WO 2005/038086    | 4/2005 |
| WO | WO 2005/038087 A1 | 4/2005 |
| WO | WO 2005/038088 A1 | 4/2005 |

**OTHER PUBLICATIONS**

Baum, et al., "Photoselective Plating of Metals for Circuitization and Top-surface Imaging", pp. 335-343, (date and publisher unavailable).  
Sone, et al., "Electroless Copper Plating Using Fe<sup>11</sup> as a Reducing Agent", Science Direct, *Electrochimica Acta* 49 (2004), pp. 233-238, [www.sciencedirect.com](http://www.sciencedirect.com), no month available.

Terskaya, et al., "Electroless Nickel and Copper Plating of Carbon Fibers with the Use of Sulfur-containing Reducing Agents", *Russian Journal of Applied Electrochemistry*, vol. 77, No. 2 (2004), pp. 236-240, no month available.

Dr. W. Kronenberg, "State of the Art for Electroless Formaldehyde-Free Copper Deposition"; 139 *Galvanotechnik* 81, No. 4; Apr. 1990; pp. 1235-1239.

\* cited by examiner

*Primary Examiner*—Helene Klemanski

(74) *Attorney, Agent, or Firm*—John J. Piskorski

(57) **ABSTRACT**

Electroless copper plating baths are disclosed. The electroless copper baths are formaldehyde free and are environmentally friendly. The electroless copper baths are stable and deposit a bright copper deposit on substrates.

**6 Claims, No Drawings**

## 1

## ELECTROLESS COPPER AND REDOX COUPLES

The present invention is directed to electroless copper compositions with redox couples. More specifically, the present invention is directed to electroless copper compositions with redox couples which are environmentally friendly.

Electroless copper plating compositions, also known as baths, are in widespread use in metallization industries for depositing copper on various types of substrates. In the manufacture of printed wiring boards, for example, the electroless copper baths are used to deposit copper into through-holes and circuit paths as a base for subsequent electrolytic copper plating. Electroless copper plating also is used in the decorative plastics industry for deposition of copper onto non-conductive surfaces as a base for further plating of copper, nickel, gold, silver and other metals as required. Typical baths which are in commercial use today contain divalent copper compounds, chelating agents or complexing agents for the divalent copper ions, formaldehyde reducing agents and various addition agents to make the bath more stable, adjust the plating rate and brighten the copper deposit. Although many of such baths are successful and are widely used, the metallization industry has been searching for alternative electroless copper plating baths that do not contain formaldehyde due to its toxic nature.

Formaldehyde is known as an eye, nose and upper respiratory tract irritant. Animal studies have shown that formaldehyde is an *in vitro* mutagen. According to a WATCH committee report (WATCH/2005/06—Working group on Action to Control Chemicals—sub committee with UK Health and Safety Commission) over fifty epidemiological studies have been conducted prior to 2000 suggested a link between formaldehyde and nasopharyngeal/nasal cancer but were not conclusive. However, more recent studies conducted by IARC (International Agency for Research on Cancer) in the U.S.A. showed that there was sufficient epidemiological evidence that formaldehyde causes nasopharyngeal cancer in humans. As a result the INRS, a French agency, has submitted a proposal to the European Community Classification and Labelling Work Group to reclassify formaldehyde from a category 3 to a category 1 carcinogen. This would make usage and handling of it more restricted, including in electroless copper formulations. Accordingly, there is a need in the metallization industry for a comparable or improved reducing agent to replace formaldehyde. Such a reducing agent must be compatible with existing electroless copper processes; provide desired capability and reliability and meet cost targets.

Hypophosphites have been suggested as a replacement for formaldehyde; however, plating rates of baths containing this compound are generally too slow.

U.S. Pat. No. 5,897,692 discloses formaldehyde free electroless plating solutions. Compounds such as boron hydride salts and dimethylamine borane (DMAB) are included as reducing agents. However, such boron containing compounds have been tried with varying degrees of success. Further, these compounds are more expensive than formaldehyde and also have health and safety issues. DMAB is toxic. Additionally, resultant borates have adverse effects on crops on release into the environment.

Accordingly, there is still a need for an electroless copper bath which is free of formaldehyde and is both stable, provides acceptable copper deposits and is environmentally friendly.

## 2

In one aspect compositions include one or more sources of copper ions, one or more chelating agents chosen from hydantoin and hydantoin derivatives and one or more redox couples.

5 In another aspect, methods include a) providing a substrate; and b) electrolessly depositing copper on the substrate using an electroless copper composition including one or more sources of copper ions, one or more chelating agents chosen from hydantoin and hydantoin derivatives and one or more redox couples.

10 In a further aspect, methods include a) providing a printed wiring board having a plurality of through-holes; b) desmearing the through-holes; and c) depositing copper on walls of the through-holes using an electroless copper composition including one or more sources of copper ions, one or more chelating agents chosen from hydantoin and hydantoin derivatives and one or more redox couples.

15 The electroless copper compositions are formaldehyde free, thus they environmentally friendly and non-carcinogenic.

20 The environmentally friendly electroless copper plating compositions are stable during storage as well as during copper deposition. Additionally, the environmentally friendly electroless copper compositions provide uniform copper deposits which have a uniform pink and smooth appearance, 25 and generally meet industry standards desired for commercially acceptable electroless copper baths. The electroless copper compositions also plate copper at commercially acceptable rates.

30 As used throughout this specification, the abbreviations given below have the following meanings, unless the context clearly indicates otherwise: g=gram; mg=milligram; ml=milliliter; L=liter; cm=centimeter; m=meter; mm=millimeter;  $\mu$ m=micron; min.=minute; ppm=parts per million;  $^{\circ}$ C.=degrees Centigrade; M=molar; g/L=grams per liter; wt %=percent by weight;  $T_g$ =glass transition temperature; and dyne=1 g-cm/second<sup>2</sup>=( $10^{-3}$  Kg) ( $10^{-2}$  m)/second<sup>2</sup>= $10^{-5}$  Newtons.

35 The terms “printed circuit board” and “printed wiring board” are used interchangeably throughout this specification. The terms “plating” and “deposition” are used interchangeably throughout this specification. A dyne is a unit of force. All amounts are percent by weight, unless otherwise noted. All numerical ranges are inclusive and combinable in any order except where it is logical that such numerical ranges 40 are constrained to add up to 100%.

45 Electroless copper compositions are formaldehyde free and are environmentally friendly. They also are stable during storage and during electroless copper deposition. The compositions provide a copper deposit with a uniform salmon pink appearance. The compositions include one or more sources of copper ions, one or more chelating agents chosen from hydantoin and hydantoin derivatives and one or more redox couples. Conventional additives also may be included in the compositions.

50 Sources of copper ions include, but are not limited to, water soluble halides, nitrates, acetates, sulfates and other organic and inorganic salts of copper. Mixtures of one or more of such copper salts may be used to provide copper ions. Examples include copper sulfate, such as copper sulfate pentahydrate,

55 copper chloride, copper nitrate, copper hydroxide and copper sulfamate. Conventional amounts of copper salts may be used in the compositions. Copper ion concentrations in the composition may range from 0.5 g/L to 30 g/L or such as from 1 g/L to 20 g/L or such as from 5 g/L to 10 g/L.

60 Chelating agents are chosen from one or more of hydantoin and hydantoin derivatives. Hydantoin derivatives include, but are not limited to, 1-methylhydantoin, 1,3-dimethylhydantoin,

toin and 5,5-dimethylhydantoin. Typically the chelating agents are chosen from hydantoin and 5,5-dimethylhydantoin. More typically, the chelating agent is 5,5-dimethylhydantoin. Such chelating agents are included in the compositions to stabilize reducing agents at alkaline pH ranges. Such chelating agents are included in the compositions in amounts of 20 g/l to 150 g/L or such as from 30 g/L to 100 g/L or such as 40 g/l to 80 g/L.

Redox couples function as reducing agents and replace the environmentally unfriendly formaldehyde. They are oxidized on catalyzed substrates and drive the deposition of copper. The cycling of a metal ion of the redox couple from a lower oxidation state to a higher oxidation state provides electrons for the reduction of copper onto the substrates. No external energy is applied to drive the deposition process. Metal salt reducing agents include, but are not limited to, metal salts from the metals of Groups IVA, IVB, VB, VIB, VIIB, VIII and IB of the Periodic Table of Elements. Oxidation states of metal ions which are strong enough reducing agents to reduce copper ions to their metallic state include, but are not limited to,  $\text{Fe}^{2+}/\text{Fe}^{3+}$ ,  $\text{Co}^{2+}/\text{Co}^{3+}$ ,  $\text{Ag}^{+}/\text{Ag}^{2+}$ ,  $\text{Mn}^{2+}/\text{Mn}^{3+}$ ,  $\text{Ni}^{2+}/\text{Ni}^{3+}$ ,  $\text{V}^{2+}/\text{V}^{3+}$ ,  $\text{Cr}^{2+}/\text{Cr}^{3+}$ ,  $\text{Ti}^{2+}/\text{Ti}^{3+}$  and  $\text{Sn}^{2+}/\text{Sn}^{4+}$ . Typically the metal is  $\text{Fe}^{2+}/\text{Fe}^{3+}$ ,  $\text{Ni}^{2+}/\text{Ni}^{3+}$ ,  $\text{Co}^{2+}/\text{Co}^{3+}$  and  $\text{Ag}^{+}/\text{Ag}^{2+}$ . More typically the metal ion is  $\text{Fe}^{2+}/\text{Fe}^{3+}$ . Anions associated with such metal ions include, but are not limited to, organic and inorganic anions such as halides, sulfates, nitrates, formates, gluconates, acetates, lactates, oxalates, tartrates, ascorbate and acetylacetone. Typical salts include iron (II) acetylacetone, iron (II) L-ascorbate, Iron (II) lactate hydrate, iron (II) oxalate dehydrate, iron (II) gluconate, iron (II) sulfate, nickel (II) chloride, cobalt (II) chloride and silver (I) nitrate. Redox couples are included in amounts of 10 g/L to 100 g/l or such as from 20 g/L to 80 g/L or such as from 30 g/L to 60 g/L.

Surfactants also may be included in the compositions. Conventional surfactants may be included in the compositions. Such surfactants include ionic, such as cationic and anionic surfactants, non-ionic and amphoteric surfactants. Mixtures of the surfactants may be used. Surfactants may be included in the compositions in amounts of 0.001 g/L to 50 g/L or such as from 0.01 g/L to 50 g/L.

Cationic surfactants include, but are not limited to, tetraalkylammonium halides, alkyltrimethylammonium halides, hydroxyethyl alkyl imidazoline, alkylbenzalkonium halides, alkylamine acetates, alkylamine oleates and alkylaminoethyl glycine.

Anionic surfactants include, but are not limited to, alkylbenzenesulfonates, alkyl or alkoxy naphthalene sulfonates, alkylidiphenyl ether sulfonates, alkyl ether sulfonates, alkylsulfuric esters, polyoxyethylene alkyl ether sulfuric esters, polyoxyethylene alkyl phenol ether sulfuric esters, higher alcohol phosphoric monoesters, polyoxyalkylene alkyl ether phosphoric acids (phosphates) and alkyl sulfosuccinates.

Amphoteric surfactants include, but are not limited to, 2-alkyl-N-carboxymethyl or ethyl-N-hydroxyethyl or methyl imidazolium betaines, 2-alkyl-N-carboxymethyl or ethyl-N-carboxymethoxyethyl imidazolium betaines, dimethylalkyl betaines, N-alkyl- $\beta$ -aminopropionic acids or salts thereof and fatty acid amidopropyl dimethylaminoacetic acid betaines.

Typically the surfactants are non-ionic. Examples of non-ionic surfactants are alkyl phenoxy polyethoxyethanols, polyoxyethylene polymers having from 20 to 150 repeating units and block copolymers of polyoxyethylene and polyoxypropylene. Surfactants may be used in conventional amounts.

Antioxidants include, but are not limited to, monohydric, dihydric and trihydric phenols in which a hydrogen atom or atoms may be unsubstituted or substituted by  $-\text{COOH}$ ,  $-\text{SO}_3\text{H}$ , lower alkyl or lower alkoxy groups, hydroquinone, catechol, resorcinol, quinol, pyrogallol, hydroxyquinol, phloroglucinol, guaiacol, gallic acid, 3,4-dihydroxybenzoic acid, phenolsulfonic acid, cresolsulfonic acid, hydroquinonsulfonic acid, catecholsulfonic acid, tiron and salts thereof. Antioxidants are included in the compositions in conventional amounts.

Alkaline compounds are included in the electroless copper plating compositions to maintain a pH of 9 and higher. A high pH is desirable because oxidation potentials for reducing agents are shifted to more negative values as the pH increases thus making the copper deposition thermodynamically favorable. Typically the electroless copper plating compositions have a pH from 10 to 14. More typically the electroless copper plating compositions have a pH from 11.5 to 13.5.

One or more compounds which provide an alkaline composition within the desired pH ranges may be used. Alkaline compounds include, but are not limited to, one or more alkaline hydroxides such as sodium hydroxide, potassium hydroxide and lithium hydroxide. Typically sodium hydroxide, potassium hydroxide or mixtures thereof are used. More typically sodium hydroxide is used. Such compounds may be included in amounts of 5 g/L to 100 g/L or such as from 10 g/L to 80 g/L.

Other additives may be included in the electroless copper compositions to tailor the compositions for optimum performance. Many of such additives are conventional for electroless copper deposition and are well known in the art.

Optional conventional additives include, but are not limited to, sulfur containing compounds such as mercaptosuccinic acid, dithiodisuccinic acid, mercaptopyridine, mercaptobenzothiazole, thiourea; compounds such as pyridine, purine, quinoline, indole, indazole, imidazole, pyrazine and their derivatives; alcohols such as alkyne alcohols, allyl alcohols, aryl alcohols and cyclic phenols; hydroxy substituted aromatic compounds such as methyl-3,4,5-trihydroxybenzoate, 2,5-dihydroxy-1,4-benzoquinone and 2,6-dihydroxynaphthalene; carboxylic acids, such as citric acid, tartaric acid, succinic acid, malic acid, malonic acid, lactic acid, acetic acid and salts thereof; amines; amino acids; aqueous soluble metal compounds such as metal chlorides and sulfates; silicon compounds such as silanes, siloxanes and low to intermediate molecular weight polysiloxanes; germanium and its oxides and hydrides; and polyalkylene glycols, cellulose compounds, alkylphenyl ethoxylates and polyoxyethylene compounds; and stabilizers such as pyridazine, methylpyridine, 1,2-di-(2-pyridyl)ethylene, 1,2-di-(pyridyl)ethylene, 2,2'-dipyridylamine, 2,2'-bipyridyl, 2,2'-bipyrimidine, 6,6'-dimethyl-2,2'-dipyridyl, di-2-pyrylketone, N,N,N',N'-tetraethylenediamine, naphthalene, 1,8-naphthyridine, 1,6-naphthyridine, tetrathiafurvalene, terpyridine, phthalic acid, isophthalic acid and 2,2'-dibenzoinic acid. Such additives may be included in the electroless copper compositions in amounts of 0.01 ppm to 1000 ppm or such as from 0.05 ppm to 10 ppm.

Other optional additives include, but are not limited to, Rochelle salts, sodium salts of ethylenediamine tetraacetic acid, nitriloacetic acid and its alkali metal salts, triethanolamine, modified ethylene diamine tetraacetic acids such as N-hydroxyethylenediamine triacetate, hydroxyalkyl substituted dialkaline triamines such as pentahydroxy propylidethylenetriamine and compounds such as N,N-dicarboxymethyl L-glutamic acid tetrasodium salt. Also s,s-ethylene diamine disuccinic acid and N,N,N',N'-tetrakis(2-hydroxypropyl)

ethylenediamine(ethylenedinitrilo)tetra-2-propanol may be included. Typically such additives function as chelating agents to keep copper (II) ions in solution. Such complexing agents may be included in the compositions in conventional amounts. Typically such complexing agents are included in amounts of from 1 g/L to 50 g/l or such as from 10 g/L to 40 g/L.

The electroless copper compositions may be used to deposit a copper on both conductive and non-conductive substrates. The electroless compositions may be used in many conventional methods known in the art. Typically copper deposition is done at temperatures of 20° C. to 60°. More typically the electroless compositions deposit copper at temperature of 30° C. to 50° C. The substrate to be plated with copper is immersed in the electroless composition or the electroless composition is sprayed onto the substrate. Conventional plating times may be used to deposit the copper onto the substrate. Deposition may be done for 5 seconds to 30 minutes; however, plating times may vary depending on the thickness of the copper desired on the substrate. Copper plating rates may range from 0.01  $\mu\text{m}/20$  minutes to 1  $\mu\text{m}/20$  minutes or such as from 0.05  $\mu\text{m}/20$  minutes to 0.5  $\mu\text{m}/20$  minutes.

Substrates include, but are not limited to, materials including inorganic and organic substances such as glass, ceramics, porcelain, resins, paper, cloth and combinations thereof. Metal-clad and unclad materials also are substrates which may be plated with the electroless copper compositions.

Substrates also include printed circuit boards. Such printed circuit boards include metal-clad and unclad with thermosetting resins, thermoplastic resins and combinations thereof, including fiber, such as fiberglass, and impregnated embodiments of the foregoing.

Thermoplastic resins include, but are not limited to, acetal resins, acrylics, such as methyl acrylate, cellulosic resins, such as ethyl acetate, cellulose propionate, cellulose acetate butyrate and cellulose nitrate, polyethers, nylon, polyethylene, polystyrene, styrene blends, such as acrylonitrile styrene and copolymers and acrylonitrile-butadiene styrene copolymers, polycarbonates, polychlorotrifluoroethylene, and vinylpolymers and copolymers, such as vinyl acetate, vinyl alcohol, vinyl butyral, vinyl chloride, vinyl chloride-acetate copolymer, vinylidene chloride and vinyl formal.

Thermosetting resins include, but are not limited to, allyl phthalate, furane, melamine-formaldehyde, phenol-formaldehyde and phenol-furfural copolymers, alone or compounded with butadiene acrylonitrile copolymers or acrylonitrile-butadiene-styrene copolymers, polyacrylic esters, silicones, urea formaldehydes, epoxy resins, allyl resins, glycercyl phthalates and polyesters.

Porous materials include, but are not limited to paper, wood, fiberglass, cloth and fibers, such as natural and synthetic fibers, such as cotton fibers and polyester fibers.

The electroless copper compositions may be used to plate both low and high  $T_g$  resins. Low  $T_g$  resins have a  $T_g$  below 160° C. and high  $T_g$  resins have a  $T_g$  of 160° C. and above. Typically high  $T_g$  resins have a  $T_g$  of 160° C. to 280° C. or such as from 170° C. to 240° C. High  $T_g$  polymer resins include, but are not limited to, polytetrafluoroethylene (PTFE) and polytetrafluoroethylene blends. Such blends include, for example, PTFE with polyphenylene oxides and cyanate esters. Other classes of polymer resins which include resins with a high  $T_g$  include, but are not limited to, epoxy resins, such as difunctional and multifunctional epoxy resins, bimaleimide/triazine and epoxy resins (BT epoxy), epoxy/polyphenylene oxide resins, acrylonitrile butadienestyrene, polycarbonates (PC), polyphenylene oxides (PPO),

polyphenylene ethers (PPE), polyphenylene sulfides (PPS), polysulfones (PS), polyamides, polyesters such as polyethyleneterephthalate (PET) and polybutyleneterephthalate (PBT), polyetherketones (PEEK), liquid crystal polymers, polyurethanes, polyetherimides, epoxies and composites thereof.

In one embodiment the electroless compositions may be used to deposit copper on walls of through-holes or vias of printed circuit boards. The electroless compositions may be used in both horizontal and vertical processes of manufacturing printed circuit boards.

In one embodiment through-holes are formed in the printed circuit board by drilling or punching or any other method known in the art. After the formation of the through-holes, the boards are rinsed with water and a conventional organic solution to clean and degrease the board followed by desmearing the through-hole walls. Typically desmearing of the through-holes begins with application of a solvent swell.

Any conventional solvent swell may be used to desmear the through-holes. Solvent swells include, but are not limited to, glycol ethers and their associated ether acetates. Conventional amounts of glycol ethers and their associated ether acetates may be used. Such solvent swells are well known in the art. Commercially available solvent swells include, but are not limited to, CIRCUPOSIT CONDITIONER™ 3302, CIRCUPOSIT HOLE PREP™ 3303 and CIRCUPOSIT HOLE PREP™ 4120 (obtainable from Rohm and Haas Electronic Materials, Marlborough, Mass.).

Optionally, the through-holes are rinsed with water. A promoter is then applied to the through-holes. Conventional promoters may be used. Such promoters include sulfuric acid, chromic acid, alkaline permanganate or plasma etching. Typically alkaline permanganate is used as the promoter. An example of a commercially available promoter is CIRCUPOSIT PROMOTER™ 4130 available from Rohm and Haas Electronic Materials, Marlborough, Mass.

Optionally, the through-holes are rinsed again with water. A neutralizer is then applied to the through-holes to neutralize any residues left by the promoter. Conventional neutralizers may be used. Typically the neutralizer is an aqueous alkaline solution containing one or more amines or a solution of 3 wt % peroxide and 3 wt % sulfuric acid. Optionally, the through-holes are rinsed with water and the printed circuit boards are dried.

After desmearing an acid or alkaline conditioner may be applied to the through-holes. Conventional conditioners may be used. Such conditioners may include one or more cationic surfactants, non-ionic surfactants, complexing agents and pH adjusters or buffers. Commercially available acid conditioners include, but are not limited to, CIRCUPOSIT CONDITIONER™ 3320 and CIRCUPOSIT CONDITIONER™ 3327 available from Rohm and Haas Electronic Materials, Marlborough, Mass. Suitable alkaline conditioners include, but are not limited to, aqueous alkaline surfactant solutions containing one or more quaternary amines and polyamines. Commercially available alkaline surfactants include, but are not limited to, CIRCUPOSIT CONDITIONER™ 231, 3325, 813 and 860 available from Rohm and Haas Electronic Materials. Optionally, the through-holes are rinsed with water after conditioning.

Conditioning is followed by microetching the through-holes. Conventional microetching compositions may be used. Microetching is designed to provide a micro-roughened copper surface on exposed copper (e.g. innerlayers and surface etch) to enhance subsequent adhesion of deposited electroless and electroplate. Microetches include, but are not limited to, 60 g/L to 120 g/L sodium persulfate or sodium or potassium

oxymonopersulfate and sulfuric acid (2%) mixture, or generic sulfuric acid/hydrogen peroxide. An example of a commercially available microetching composition includes CIRCUPOSIT MICROETCH™ 3330 available from Rohm and Haas Electronic Materials. Optionally, the through-holes are rinsed with water.

A pre-dip is then applied to the microetched through-holes. Examples of pre-dips include 2% to 5% hydrochloric acid or an acidic solution of 25 g/L to 75 g/L sodium chloride. Optionally, the through-holes are rinsed with cold water.

A catalyst is then applied to the through-holes. Any conventional catalyst may be used. The choice of catalyst depends on the type of metal to be deposited on the walls of the through-holes. Typically the catalysts are colloids of noble and non-noble metals. Such catalysts are well known in the art and many are commercially available or may be prepared from the literature. Examples of non-noble metal catalysts include copper, aluminum, cobalt, nickel, tin and iron. Typically noble metal catalysts are used. Suitable noble metal colloid catalysts include, for example, gold, silver, platinum, palladium, iridium, rhodium, ruthenium and osmium. More typically, noble metal catalysts of silver, platinum, gold and palladium are used. Most typically silver and palladium are used. Suitable commercially available catalysts include, for example, CIRCUPOSIT CATALYST™ 3344 and CATA-POSIT™ 44 available from Rohm and Haas Electronic Materials. The through-holes optionally may be rinsed with water after application of the catalysts.

The walls of the through-holes are then plated with copper with an electroless composition as described above. Typically copper is plated on the walls of the through-holes. Plating times and temperatures are also described above.

After the copper is deposited on the walls of the through-holes, the through-holes are optionally rinsed with water. Optionally, anti-tarnish compositions may be applied to the metal deposited on the walls of the through-holes. Conventional anti-tarnish compositions may be used. Examples of anti-tarnish compositions include ANTI TARNISH™ 7130 and CUPRATECT™ 3 (obtainable from Rohm and Haas Electronic Materials). The through-holes may optionally be rinsed by a hot water rinse at temperatures exceeding 30° C. and then the boards may be dried.

In an alternative embodiment the through-holes may be treated with an alkaline hydroxide solution after desmear to prepare the through-holes for electroless deposition of copper. This alternative embodiment for plating through-holes or vias is typically used when preparing high  $T_g$  boards for plating. The alkaline hydroxide solution contacts the through-holes for 30 seconds to 120 seconds or such as from 60 seconds to 90 seconds. Application of the alkaline hydroxide composition between the desmearing and plating the through-holes provides for good coverage of the through-hole walls with the catalyst such that the copper covers the walls. The alkaline hydroxide solution is an aqueous solution of sodium hydroxide, potassium hydroxide or mixtures thereof. The hydroxides are included in amounts of 0.1 g/L to 100 g/L or such as from 5 g/L to 25 g/L. Typically the hydroxides are included in the solutions in amounts of 15 g/L to 20 g/L. Typically the alkaline hydroxide is sodium hydroxide. If the alkaline hydroxide solution is a mixture of sodium hydroxide and potassium hydroxide, the sodium hydroxide and potassium hydroxide are in a weight ratio of 4:1 to 1:1, or such as from 3:1 to 2:1.

Optionally one or more surfactants may be added to the alkaline hydroxide solution. Typically the surfactants are non-ionic surfactants. The surfactants reduce surface tension to enable proper wetting of the through-holes. Surface tension

after application of the surfactant in the through-holes ranges from 25 dynes/cm to 50 dynes/cm, or such as from 30 dynes/cm to 40 dynes/cm. Typically the surfactants are included in the formulation when the alkaline hydroxide solution is used to treat small through-holes to prevent flaring. Small through-holes typically range in diameter of 0.2 mm to 0.5 mm. In contrast, large through-holes typically range in diameter of 0.5 mm to 1 mm. Aspect ratios of through-holes may range from 1:1 to 20:1.

Surfactants are included in the alkaline hydroxide solutions in amounts of 0.05 wt % to 5 wt %, or such as from 0.25 wt % to 1 wt %. Suitable non-ionic surfactants include, for example, aliphatic alcohols such as alkoxylates. Such aliphatic alcohols have ethylene oxide, propylene oxide, or combinations thereof, to produce a compound having a polyoxyethylene or polyoxypropylene chain within the molecule, i.e., a chain composed of recurring (—O—CH<sub>2</sub>—CH<sub>2</sub>) groups, or chain composed of recurring (—O—CH<sub>2</sub>—CH—CH<sub>3</sub>) groups, or combinations thereof. Typically such alcohol alkoxylates are alcohol ethoxylates having carbon chains of 7 to 15 carbons, linear or branched, and 4 to 20 moles of ethoxylate, typically 5 to 40 moles of ethoxylate and more typically 5 to 15 moles of ethoxylate.

Many of such alcohol alkoxylates are commercially available. Examples of commercially available alcohol alkoxylates include, for example, linear primary alcohol ethoxylates such as NEODOL 91-6, NEODOL 91-9 (C<sub>9</sub>-C<sub>11</sub> alcohols having an average of 6 to 9 moles of ethylene oxide per mole of linear alcohol ethoxylate) and NEODOL 1-73B (C<sub>11</sub> alcohol with an average blend of 7 moles of ethylene oxide per mole of linear primary alcohol ethoxylate). Both are available from Shell Oil Company, Houston Tex.

After the through-holes are treated with the alkaline hydroxide solution, they may be treated with an acid or alkaline conditioner. The through-holes are then micro-etched and applied with a pre-dip followed by applying a catalyst. The through-holes are then electrolessly plated with copper.

After the through-holes are plated with copper, the substrates may undergo further processing. Further processing may include conventional processing by photoimaging and further metal deposition on the substrates such as electrolytic metal deposition of, for example, copper, copper alloys, tin and tin alloys.

While not being bound by theory, the hydantoin and the hydantoin derivatives enable a controlled autocatalytic deposition of copper on substrates using the redox couples at an alkaline pH. These hydantoin and hydantoin derivatives stabilize the copper ions in solution and prevent formation of copper precipitates, i.e. copper oxides and hydroxides, which typically form at an alkaline pH in the presence of the redox couples. Such copper precipitate formation destabilizes the electroless copper compositions and compromises the deposition of copper on substrates. The inhibition of the copper precipitate formation enables the process to operate at high pH ranges where copper deposition is thermodynamically favorable.

The electroless copper compositions are free of formaldehyde and are environmentally friendly. They are stable during storage and during electroless deposition. They deposit a uniform copper layer on a substrate which is uniform salmon pink appearance. The uniform salmon pink appearance typically indicates that the copper deposit is smooth and fine grained. A fine grain is desired for good mechanical properties and coverage. A dark deposit may indicate coarseness, roughness and nodular formation, which is unacceptable to the metallization industry.

The following examples are not intended to limit the scope of the invention but are intended to further illustrate it.

## EXAMPLE 1

Three aqueous electroless copper compositions included iron (II) gluconate and 5,5-dimethylhydantoin. The electroless copper compositions were free of formaldehyde and were environmentally friendly. They were tested for their stability and quality of their copper deposits. Each aqueous electroless composition included at least 7 g/L of copper chloride ( $\text{CuCl}_2 \cdot 2\text{H}_2\text{O}$ ), 63 g/L of iron (II) gluconate and 64 g/L of 5,5-dimethylhydantoin.

Electroless copper compositions 2 and 3 included a complexing agent. Composition 1 was free of complexing agent. Composition 2 included 36 g/L of ethylenediamine tetraacetic acid. Composition 3 included the complexing agent N,N-dicarboxymethyl L-glutamic acid tetrasodium salt at 82 mL/L.

The temperature of the compositions was maintained at 55° C. and a pH of 13.2 during electroless copper deposition. Copper was deposited on substrates for 20 minutes. The substrates used were unclad FR4 epoxy/glass laminates with dimensions 1.5 inches×1.5 inches (2.54 cm/inch). The printed circuit boards were obtained from Isola Laminate Systems Corp., LaCrosse Wis. The process was as follows:

1. The surface of each laminate was immersed in an aqueous bath containing 5% of the aqueous acid conditioner CIRCUPOSIT CONDITIONER™ 3327 for 6 minutes at 50° C.
2. Each laminate was then rinsed with cold water for 6 minutes.
3. A pre-dip was then applied to each laminate for 1 minute at room temperature. The pre-dip was Pre-dip™ 3340 obtainable from Rohm and Haas Electronic Materials.
4. The laminates were then primed for 6 minutes at 40° C. with a catalyst for electroless copper metallization. The laminates were primed by immersing the laminates in the catalyst. The catalyst was CIRCUPOSIT CATALYST™ 3344.
5. The laminates were then rinsed with cold water for 5 minutes.
6. Each laminate was then immersed in one of the electroless copper plating compositions described above for copper metal deposition. Copper metal deposition was done over 20 minutes. No insoluble copper salt precipitate was observed during copper plating. Accordingly, the compositions were stable.
7. The copper plated laminates were then rinsed with cold water for 2 minutes.
8. Each copper plated laminate was then rinsed with deionized water for one minute.
9. Each copper plated laminate was then placed into a conventional convection oven and dried for 20 minutes at 105° C.
10. After drying each copper plated laminate was placed in a conventional laboratory dessicator for 20 minutes or until it cooled to room temperature.
11. After drying each copper plated laminate was observed for the quality of the copper deposit. The laminates plated with electroless copper compositions 2 and 3 had a good appearance. Electroless copper composition 1 had a dark brown appearance (see Table below).
12. Each copper plated laminate was then weighed on a conventional balance and recorded.
13. After weighing and recording the weight of each laminate, the copper deposit was etched from each laminate by immersing the laminate in a 3% sulfuric acid/3% hydrogen peroxide solution.
14. Each laminate was then rinsed with cold water for 3 minutes.

- 5 15 20 25 30 35 40 45 50 55 60 65 70 75 80 85 90 95
15. Each laminate was then put back in the oven for 20 minutes at 105° C.
16. The laminates were then placed in a dessicator for 20 minutes or until it reached room temperature.
17. The laminates were then weighed and the weight difference before etching and after etching was determined. The weight difference was used to determine the plating rates. The plating rates for each laminate are in the table below.

TABLE 2

| COMPOSITION | STABILITY      | RATE<br>(μm/20 minutes) | APPEARANCE  |
|-------------|----------------|-------------------------|-------------|
| 1           | No precipitate | 0.016                   | Dark brown  |
| 2           | No precipitate | 0.312                   | Salmon pink |
| 3           | No precipitate | 0.320                   | Salmon pink |

All except one of the copper deposits appeared salmon pink, which indicated that such copper deposits were uniform with a fine grain and suitable for industrial application. The dark brown appearance of the deposit from composition 1 may have been caused by passivation/oxidation of the copper deposit.

## EXAMPLE 2

Two aqueous electroless copper compositions included iron (II) gluconate and hydantoin. They were tested for their stability and quality of their copper deposits. Each aqueous electroless composition included at least 7 g/L of copper chloride ( $\text{CuCl}_2 \cdot 2\text{H}_2\text{O}$ ), 63 g/L of (II) gluconate and 50 g/L of hydantoin. Composition 1 also included 82 mL/L N,N-dicarboxymethyl L-glutamic acid tetrasodium salt. The electroless copper compositions were formaldehyde free and environmentally friendly.

The temperature of the compositions was maintained at 55° C. and a pH of 13.2 during electroless copper deposition. Copper was deposited on substrates for 20 minutes. The substrates were two unclad FR4 epoxy/glass laminates with dimensions 1.5 inches×1.54 inches (2.54 cm/inch). The laminates were obtained from Isola Laminate System Corp., LaCrosse Wis. The process was the same as described in Example 1 above. The results of the tests are in the table below.

TABLE 3

| COMPOSITIONS | STABILITY       | RATE<br>(μm/20 minutes) | APPEARANCE  |
|--------------|-----------------|-------------------------|-------------|
| 1            | Stable          | 0.528                   | Salmon pink |
| 2            | Red precipitate | 0.00                    | No plating  |

Composition 1 was stable during copper deposition and deposited a uniform copper layer with fine grains on the FR4 epoxy glass laminate. Accordingly, composition 1 deposited an industrially acceptable copper layer on the laminate.

Composition 2 was unstable as evidenced by a red precipitate in the electroless composition. Further, no copper plating was observed.

What is claimed is:

1. A composition comprising one or more sources of copper ions, one or more chelating agents selected from the group consisting of hydantoin and hydantoin derivatives and one or more redox couples, the redox couples comprise metal ions selected from the group consisting of Groups IVA, IVB, VB, VIB, VIIIB, VIII and IB of the periodic Table of Elements.

**11**

2. The composition of claim 1, wherein the hydantoin derivatives are selected from the group consisting of 1-methylhydantoin, 1,3-dimethylhydantoin and 5,5-dimethylhydantoin.

3. The composition of claim 1, wherein anions associated with the metal ions are selected from the group consisting of organic and inorganic ions.

4. The composition of claim 3, wherein the anions are selected from the group consisting of halides, nitrates, sulfates, formates, gluconates, acetates, lactates, oxalates, tartrates, ascorbate and acetylacetone. 10

5. A method comprising:

- a) providing a substrate; and
- b) electrolessly depositing copper on the substrate with an 15 electroless copper composition comprising one or more sources of copper ions, one or more chelating agents selected from the group consisting of hydantoin and

**12**

hydantoin derivatives and one or more redox couples, the redox couples comprise metal ions selected from the group consisting of Groups IVA, IVB, VB, VIB, VIIIB, VIII and IB of the periodic Table of Elements.

6. A method comprising:

- a) providing a printed wiring board comprising a plurality of through-holes;
- b) desmearing the through-holes; and
- c) depositing copper on walls of the through-holes with an electroless copper composition comprising one or more sources of copper ions, one or more chelating agents selected from the group consisting of hydantoin and hydantoin derivatives and one or more redox couples, the redox couples comprise metal ions selected from the group consisting of Groups IVA, IVB, VB, VIB, VIIIB, VIII and IB of the periodic Table of Elements.

\* \* \* \* \*